

# UNITED STATES PATENT OFFICE.

NELSON S. WHITE, OF CANTON, MASSACHUSETTS.

## MANUFACTURE OF METALLIC-SURFACED INDIA-RUBBER FABRIC.

SPECIFICATION forming part of Letters Patent No. 278,206, dated May 22, 1883.

Application filed August 11, 1882. (Specimens.)

To all whom it may concern:

Be it known that I, NELSON S. WHITE, of Canton, in the county of Norfolk and State of Massachusetts, a citizen of the United States, have invented a new and useful Improvement in the Manufacture of Metallic-Surfaced India-Rubber or Gutta-Percha Fabric, of which the following is a full, clear, and exact description.

10 My invention relates to the manufacture of bronze-finished fabrics; and it consists in coating a close-textured fabric with a composition of plastic india-rubber, gutta-percha, or other like material adapted to become set or fixed by evaporation or heat, and upon and into the surface of which while yet plastic the bronze powder or laminæ is spread and incorporated by pressure.

I prefer to use in practicing my invention 20 either of the compositions described in Letters Patent Nos. 202,427, 238,372, and 238,496, granted Charles A. Evans, in about the proportion therein named, with the exception that the coloring matter or material may be omitted therefrom, although, of course, I do not wish it to be understood that it may not be used, if desired. The compositions described in said Letters Patent consist, substantially, 25 of india-rubber or gutta-percha, or both, dissolved in naphtha, and a suitable filling material used for giving body to the mixture, cheapening and coloring it; but, in lieu of a plastic compound of this nature containing an evaporating agent, the evaporation of which 30 fixes or sets the rubber or gutta-percha, I may use a plastic compound adapted to be set or fixed by heat. Any suitable fabric may be used, and I mention particularly cloth, leather, and paper as among the more desirable.

40 The composition is applied in one or more coats to the fabric, and while plastic or before it sets or becomes fixed the bronze powder or laminæ spread upon the surface of the last coating in a uniform layer, and is rolled or 45 otherwise compressed therein, and the fixing or setting of the composition by evaporation or by heat permanently fastens the powder or laminæ to the fabric.

It will be obvious, of course, that the plastic composition will take or permit of a large

amount of the powder being used, and that the powder or laminæ, when worked into its surface, is very securely fastened or held, so that a very permanent and brilliant bronze finish is obtained.

55 It will be seen, also, that a holding medium of the character described not only serves to fasten large quantities of the powder or laminæ to the fabric in a substantial manner, but, owing to its elasticity or flexibility, it permits the fabric to be folded, stretched, or manipulated without damaging or in any way disturbing the bronze finish.

It will be seen, also, that a holding medium of the character described not only serves to fasten large quantities of the powder or laminæ to the fabric in a substantial manner, but, owing to its elasticity or flexibility, it permits the fabric to be folded, stretched, or manipulated without damaging or in any way disturbing the bronze finish.

I prefer to use, for obtaining brilliancy of 60 finish, bronzing material in the shape of laminæ rather than powder, and to apply it dry, although it may be applied in a liquid form.

The fabric may be pebbled during the course of its manufacture or after the powder has been applied, if desired.

70 It will be seen that the plastic rubber or gutta-percha compound prepared to be set or fixed by heat or evaporation acts as a mordant in fixing and setting the bronze powder or laminæ, which is incorporated therewith.

Having thus fully described my invention, I claim and desire to secure by Letters Patent of the United States—

1. A close-textured fabric coated with a plastic composition containing rubber, gutta-percha, or both, adapted to be set by evaporation or heat, upon and in which coating bronze powder or laminæ is spread and embedded, all substantially as and for the purposes described.

80 2. As a means of bronzing fabrics, a plastic composition or solution containing india-rubber or gutta-percha, or both, adapted to become fixed or set by heat or evaporation, spread upon the fabric, and in which the bronze powder or laminæ is incorporated by pressure, all substantially as and for the purposes described.

90 3. The combination of a close-textured fabric, a coating of india-rubber and gutta-percha, or either compound, and a surfacing of bronze powder or laminæ incorporated by pressure into the coating while the same is plastic, all substantially as and for the purposes described.

55

65

70

75

85

100

4. The process of bronzing fabrics, consisting in coating the fabric with one or more layers of plastic gutta-percha or india-rubber compound, or a compound of like nature adapted to be set or fixed by evaporation or by heat, and a bronze powder or laminae applied to the upper surface of the last layer

while plastic and united thereto by pressure, all substantially as and for the purposes described.

NELSON S. WHITE.

Witnesses:

F. F. RAYMOND, 2d,  
W. CLIFTON FOGG.